

## UNITED STATES PATENT OFFICE

2,203,826

CATALYTIC DEHYDROGENATION OF  
HYDROCARBONS

Vasili Komarewsky, Chicago, Ill., assignor to  
Universal Oil Products Company, Chicago, Ill.,  
a corporation of Delaware

No Drawing. Application December 31, 1937,  
Serial No. 182,808

12 Claims. (Cl. 260—668)

This invention is concerned with reactions involving the dehydrogenation of aliphatic hydrocarbons and refers more specifically to the production of cyclic hydrocarbons by reactions involving the dehydrogenation of paraffinic hydrocarbons containing at least six carbon atoms in straight chain arrangement to produce aromatics. The process is therefore primarily applicable to normally liquid aliphatic hydrocarbon materials consisting either of pure compounds or mixtures.

In the ordinary thermal treatment of aliphatic hydrocarbons, it is apparent that the primary reactions involve a loss of hydrogen with the formation of mono-olefins and that further conversion involves a further loss of hydrogen and forms di-olefins and miscellaneous cyclic hydrocarbons possibly resulting from the condensation and cyclization of highly unsaturated aliphatic residues. In such cracking reactions, however, there is a considerable spread in the products which include normally gaseous hydrocarbons and liquid hydrocarbons running from the very lightest which can exist as liquid under ordinary conditions up to high boiling condensation products and tars. Under intensive cracking conditions there will be produced definite yields of aromatic hydrocarbons such as benzene and toluene although these yields are seldom high enough to make this method of aromatic production one of commercial importance. The present process deals with the application of specific catalysts to the production of aromatics from aliphatic hydrocarbons, including both paraffins and mono-olefins.

In one specific embodiment the present invention comprises a process for the manufacture of aromatic hydrocarbons by subjecting the vapors of aliphatic hydrocarbons containing at least six carbon atoms in straight chain arrangement to contact with granular catalysts comprising aluminum oxide, chromium sesqui-oxide, and reduced nickel at temperatures, pressures, and rates most conducive to the formation of the desired products.

The type of reactions which are brought about by the use of the specific catalysts to be presently discussed are included in the generic term of "dehydrocyclization" and are typified by the reactions shown below in which formation of benzene, toluene, and xylene from normal hexane,

normal heptane, and normal octane are shown.



In the structural equations shown above no attempt has been made to portray possible intermediate products such as, for example, the corresponding mono-olefins which evidently are formed as primary products of dehydrogenation, or other products such as di-olefins which might result from further dehydrogenation reactions, and no account is taken of the fact that the cyclization may occur before extensive dehydrogenation of the original molecule. Under the preferred conditions of operation, conditions are so regulated that maximum yields of the aromatic hydrocarbons are obtained. It is evident from the above structural equations which have been substantiated by experimental work that end methyl groups of compounds having more than 6 carbon atoms in straight chain arrangement appear in the benzene ring. With higher molecular weight paraffins containing more than eight carbon atoms in straight chain arrangement, the reactions ordinarily become more complex, and with hydrocarbons from 10 to 12 carbon atoms in linear arrangement there is some tendency for the formation of naphthalene.

The catalysts which are used according to the present invention to bring about dehydrogenation and cyclization of aliphatic hydrocarbons comprise, as already stated, mixtures of aluminum oxide, chromium sesqui-oxide, and re-

duced nickel. The proportions of these ingredients may be varied considerably though in general the aluminum oxide will be in major proportion and the chromium oxide and nickel in minor proportion. An effective catalyst whose preparation will be described in a succeeding paragraph consists of approximately 65% by weight of aluminum oxide ( $Al_2O_3$ ), 30% by weight of chromium sesquioxide ( $Cr_2O_3$ ), and 5% 5 reduced nickel. The relative proportions of the chromium oxide and the reduced nickel may be varied somewhat depending upon the hydrocarbon treated to produce optimum yields of aromatics. As a rule the amount of nickel present 10 on the catalyst will be substantially less than the amount of chromium oxide and the total amount of nickel will be definitely a minor amount of the total weight of the catalyst.

The preferred catalysts are prepared by a special and specific procedure which may be briefly summarized as follows. An aqueous solution containing the nitrates of chromium and aluminum in proper relative proportions for producing a catalyst containing the alumina and chromia in the proper ratio is treated with an alkali metal hydroxide such as sodium hydroxide to first precipitate the hydroxides of aluminum and chromium. These hydroxides are then redissolved in just the requisite excess of alkali to 20 form a clear solution which will then comprise sodium aluminate, and sodium chromite. To this solution a composite solution containing nickel nitrate and either ammonium nitrate or nitric acid is added to form a mixed precipitate of nickel, chromium, and aluminum hydroxides. The precipitate is washed with water to the removal of substantially all adsorbed salts and then dried and reduced in a current of hydrogen at 25 gradually increasing temperatures up to 425-450° C. It has been found that under these conditions substantially all of the chromium oxides are reduced to chromium sesquioxide and that the nickel oxides are substantially all reduced to metallic nickel. By this method of preparation 30 it is obvious that the components of the catalysts are in a state of extremely intimate admixture so that each component is able to best exert its promoting effect upon the other components.

The subject of promoter catalysis is one which 35 is difficult to analyze and most of the knowledge thereof is on an empirical basis. In the present instance the experimental evidence indicates that the effect of small additions of nickel is to greatly accentuate the dehydrogenating properties of alumina-chromia mixtures so that dehydrocyclization reactions are effected at lower temperatures than when employing chromium oxides alone, alumina-chromia catalysts alone, or reduced nickel alone or on supports such as 40 alumina.

In operating to produce aromatics from paraffins or mono-olefins according to the present process, the granular catalysts consisting of particles of an approximate mesh of from 4 to 20 45 are placed in catalyst chambers and the vaporized aliphatic hydrocarbon is passed through the granular mass at temperatures of the order of from 400 to 500° C. which is considerably lower than those which are generally used with oxide 50 catalysts or those comprising alumina or other refractory oxides promoted by lower oxides of metals such as chromium. The pressures employed are substantially atmospheric and the rates will be varied in accordance with the type 55 of hydrocarbon undergoing treatment and the

character of the aromatic products desired. The products from the treatment will include fixed gases of which a large portion will be hydrogen, a certain amount of low boiling hydrocarbons, some olefins including both mono and di-olefins, and preponderating amounts of aromatics when conditions have been suitably chosen for the conversion. The aromatic products may be separated from unconverted aliphatic hydrocarbons and the latter returned for further conversion in 10 admixture with fresh charge.

The following example is given of the formation of aromatics from normal paraffinic hydrocarbons to show the value of the process in comparison with other processes having the 15 same object, although not with the intent of unduly circumscribing the scope of the invention.

The catalyst for the reaction was prepared as follows. An aqueous solution containing 175 20 parts by weight of chromium nitrate,



and 375 parts by weight of aluminum nitrate, 25



was treated with an aqueous solution of sodium hydroxide to primarily precipitate the hydroxides of aluminum and chromium and then redissolve 30 the primary precipitate to form a solution of sodium aluminate and sodium chromite. To the clear solution, 35 parts by weight of nickel nitrate and 400 parts by weight of ammonium nitrate in joint solution were added slowly with 35 stirring to form a mixed precipitate of nickel, chromium, and aluminum hydroxides. The precipitate was washed by decantation and mechanical filtration, dried at a temperature of 110° C. and finally reduced in a current of hydrogen at 40 gradually increasing temperatures from about 200 to 450° C. The granulation of the material was effected after the drying stage and before reduction.

Using the catalyst prepared as above which 45 comprised approximately 65% by weight of aluminum oxide, 30% by weight of chromium sesquioxide, and 5% nickel, normal heptane was vaporized and passed over the granular catalyst 50 at a temperature of 450° C. The vapors were pre-heated to this temperature, and the temperature of the catalyst bed was maintained by exterior heating on account of the endothermic character of the reaction. In a single pass through this catalyst the total liquid recovery was 62% by volume, the yield of toluene based on the charging material was 31% and the yield of olefins (principally a mixture of heptenes) was 10.3%. Using a catalyst comprising 70% by weight of alumina and 30% by weight of chromium sesquioxide without nickel the liquid recovery at the same temperature of 450° C. was 75%, the yield of toluene based on the charge was 24%, and the yield of heptenes was 9%. It is thus seen that the use of nickel in conjunction with chromium 60 sesquioxide gives definitely increased yields of toluene over the yields obtained when employing alumina-chromia catalysts without nickel. The increased activity of the alumina-chromia-nickel catalyst is also shown by the lower liquid recovery 65 indicating a higher degree of gasification.

The nature of the present invention is apparent from the foregoing specification including both descriptive and numerical sections neither of which is intended to be unduly limiting.

I claim as my invention:

1. A process for dehydrogenating aliphatic hydrocarbons which comprises subjecting the same to dehydrogenating conditions in the presence of a catalyst comprising a major proportion of alumina and minor proportions of chromium sesquioxide and nickel.
2. A process for dehydrogenating paraffinic hydrocarbons which comprises subjecting the same to dehydrogenating conditions in the presence of a catalyst comprising a major proportion of alumina and minor proportions of chromium sesquioxide and nickel.
3. A process for dehydrogenating mono-olefinic hydrocarbons which comprises subjecting the same to dehydrogenating conditions in the presence of a catalyst comprising a major proportion of alumina and minor proportions of chromium sesquioxide and nickel.
4. A process for dehydrogenating aliphatic hydrocarbons which comprises subjecting the same to dehydrogenating conditions in the presence of a catalyst comprising a major proportion of alumina and minor proportions of chromium sesquioxide and nickel, the sesquioxide being in greater weight than the nickel.
5. A process for dehydrogenating paraffinic hydrocarbons which comprises subjecting the same to dehydrogenating conditions in the presence of a catalyst comprising a major proportion of alumina and minor proportions of chromium sesquioxide and nickel, the sesquioxide being in greater weight than the nickel.
6. A process for dehydrogenating mono-olefinic hydrocarbons which comprises subjecting the same to dehydrogenating conditions in the presence of a catalyst comprising a major proportion of alumina and minor proportions of chromium sesquioxide and nickel, the sesquioxide being in greater weight than the nickel.
7. A process for producing aromatics from aliphatic hydrocarbons of at least six carbon atoms in straight chain arrangement, which comprises subjecting the aliphatic hydrocarbons to dehydrogenating and cyclizing conditions in the presence of a catalyst comprising a major proportion of alumina and minor proportions of chromium sesquioxide and nickel.
8. A process for producing aromatics from paraffinic hydrocarbons of at least six carbon atoms in straight chain arrangement, which comprises subjecting the paraffinic hydrocarbons to dehydrogenating and cyclizing conditions in the presence of a catalyst comprising a major proportion of alumina and minor proportions of chromium sesquioxide and nickel.
9. A process for producing aromatics from mono-olefinic hydrocarbons of at least six carbon atoms in straight chain arrangement, which comprises subjecting the mono-olefinic hydrocarbons to dehydrogenating and cyclizing conditions in the presence of a catalyst comprising a major proportion of alumina and minor proportions of chromium sesquioxide and nickel.
10. A process for producing aromatics from aliphatic hydrocarbons of at least six carbon atoms in straight chain arrangement, which comprises subjecting the aliphatic hydrocarbons to dehydrogenating and cyclizing conditions in the presence of a catalyst comprising a major proportion of alumina and minor proportions of chromium sesquioxide and nickel, the sesquioxide being in greater weight than the nickel.
11. A process for producing aromatics from paraffinic hydrocarbons of at least six carbon atoms in straight chain arrangement, which comprises subjecting the paraffinic hydrocarbons to dehydrogenating and cyclizing conditions in the presence of a catalyst comprising a major proportion of alumina and minor proportions of chromium sesquioxide and nickel, the sesquioxide being in greater weight than the nickel.
12. A process for producing aromatics from mono-olefinic hydrocarbons of at least six carbon atoms in straight chain arrangement, which comprises subjecting the mono-olefinic hydrocarbons to dehydrogenating and cyclizing conditions in the presence of a catalyst comprising a major proportion of alumina and minor proportions of chromium sesquioxide and nickel, the sesquioxide being in greater weight than the nickel.

VASILI KOMAREWSKY.